

No. 722,050.

PATENTED MAR. 3, 1903

F. SCHaab.  
PROCESS OF PRINTING COTTON.

APPLICATION FILED JAN. 26, 1902.

NO MODEL.



WITNESSES:

Walter Koehlein  
Henry Schubier.

INVENTOR

Franz Schaab  
BY  
Graesbach

ATTORNEYS

# UNITED STATES PATENT OFFICE.

FRANZ SCHaab, OF TRIER, GERMANY.

## PROCESS OF PRINTING COTTON.

SPECIFICATION forming part of Letters Patent No. 722,050, dated March 3, 1903.

Application filed January 25, 1902. Serial No. 91,252. (No specimens.)

*To all whom it may concern:*

Be it known that I, FRANZ SCHaab, of Trier, in the Empire of Germany, have invented certain new and useful Improvements in Processes of Printing Cotton Fabrics, of which the following is a specification.

This invention relates to an improved process for printing fabrics of cotton or other vegetable fiber in white or colored designs. It was heretofore impossible to produce by the employment of dyestuffs used in an alkaline solution—for example, the so-called "sulfur dyes"—these effects, for the reason that the resists known and employed did not possess sufficient resistance to withstand the continuous passage through the dye-baths.

The object of the present invention is to provide a process by which this difficulty is overcome; and for this purpose the invention consists in printing the fabric with a suitable resist of any common or well-known composition—such, for instance, as that hereinabove described—treating said resist imprinted on the goods with a solution of a suitable alkali, then thoroughly drying the goods, and then dyeing the same in an alkaline bath.

When a resist of the ordinary composition is printed on cotton or other vegetable fiber and then subjected to the action of a solution of an alkali carbonate and subsequently dried, it is rendered capable of resisting successfully the continuous hydrosulfit-soda (hydrosulfit-natron) bath. In place of an alkali carbonate a caustic-alkali or other alkaline salt or salts may be used. In all cases, however, it is necessary for the production of an effective resist that after the treatment of the resist by the alkaline solution the goods are thoroughly dried. When the resist is only partly dry or moist, it does not sufficiently resist the influence of the bath, and the desired result is not obtained. For the resist a mixture of soluble lead or copper salts, common pipe-clay, lead sulfate, and a thickening agent, such as any suitable gum, can be used. In place of the lead or copper salts other salts, such as zinc or manganese salts, may be employed and yield similar results. After the fabric has been printed by suitable rolls with the resist and treated by splashing thoroughly with the alkaline solution and

then completely dried the goods are dyed in an alkaline bath in the usual manner with indigo or other color. The undyed portions protected by the resist appear in clear white and produce clear effects. Before the fabrics are passed through the indigo-bath they can be dyed with sulfur dyes, or they may be first dyed in the indigo-bath and then again dyed with sulfur dyestuffs. In place of the white effect on the blue ground a yellow effect can be produced when the fabrics are passed after the dyeing through a solution of bichromate of potash.

In the accompanying drawing, which shows a piece of goods dyed according to the improved process, *a* indicate portions protected by the resist, and *b* the portion dyed in the dye-bath.

In practically carrying out my improved process the cotton fabric is first printed in any approved manner with a resist, which may be of the following composition: twenty kilograms of lead sulfate in paste form, twelve and one-half kilograms of lead nitrate, seven and one-half kilograms of sugar of lead, three kilograms cupric sulfate, six liters cupric nitrate, three kilograms alum, three kilograms leiogomme, four kilograms lightly-burned starch, eight kilograms of a solution of suitable gum, and one-half kilogram tallow. The fabric is dried after printing and then saturated, as by spraying or splashing, with a concentrated aqueous solution of potash, (specific gravity 1.54.) It is then thoroughly dried and then passed through a dye-bath, which contains, per one hundred liters, two kilograms of a suitable blue, such as that known as "immedial blue CR," one kilogram sodium sulfid, one-half kilogram soda-lye of 40° Baumé, and two kilograms common salt. The fabric is then steamed, if necessary, washed, acidified, and dried.

If the fabrics are to be dyed also in indigo, they are not required to be washed and acidified before dyeing with indigo. The latter step can be accomplished directly in the usual hydrosulfit-soda bath. After the indigo-bath is applied to the fabrics they are acidified, washed, and dried.

The process described produces a blue ground with white designs. If designs in

other colors, such as yellow or orange, are desired, this effect is obtained by passing the fabric subsequently through a bath of bichromate solution in the well-known manner.

5 In the foregoing process the same effects may be obtained by substituting for potash soda or a solution of caustic soda.

It is preferable to dry the goods, after the treatment with the alkaline carbonate, quickly, as by the use of high heat.

Having thus described my invention, I claim as new and desire to secure by Letters Patent—

1. The process herein described of printing cotton fabrics, which consists in printing on the fabric a resist containing metallic salts, then spraying the fabric with a solution of an alkaline carbonate, then thoroughly drying the fabric, then dyeing the same with a 15 sulfur dyestuff, and subsequently dyeing the

same with indigo in an alkaline bath, substantially as set forth.

2. The process herein described of printing cotton fabrics, which consists in printing on the fabric a resist containing metallic salts, 25 then spraying the fabric with a solution of an alkaline carbonate, then thoroughly drying the fabric, then dyeing the same with a sulfur dyestuff in an alkaline bath, then dyeing the same with indigo in an alkaline bath, 30 and then passing the same through a bichromate solution, substantially as set forth.

In testimony that I claim the foregoing as my invention I have signed my name in presence of two subscribing witnesses.

FRANZ SCHaab.

Witnesses:

ADOLPH SIMPLE,  
CARL SCHMITT.